

June 26, 1923.

C. H. HOWARD

1,460,356

REINFORCED PAPER STRIP

Filed April 15, 1920



Fig. 3



Inventor:  
Charles H. Howard

By R. H. Davis,  
Attorney

## UNITED STATES PATENT OFFICE.

CHARLES H. HOWARD, OF SAUGUS, MASSACHUSETTS, ASSIGNOR TO PAPER PRODUCTS MACHINE COMPANY, OF BOSTON, MASSACHUSETTS, A CORPORATION OF MASSACHUSETTS.

## REINFORCED-PAPER STRIP.

Application filed April 15, 1920. Serial No. 374,134.

To all whom it may concern:

Be it known that I, CHARLES H. HOWARD, a citizen of the United States, and a resident of Saugus, county of Essex, and State of Massachusetts, have invented an Improvement in Reenforced-Paper Strips, of which the following description, in connection with the accompanying drawings, is a specification, like characters on the drawings representing like parts.

The invention to be hereinafter described relates to composite reenforced fabrics, and more particularly to plural ply fabrics reenforced by unspun fibres, such, for example, as ramie, hemp, sisal, flax and other forms of fibres.

The preparation of the natural fibre in its unspun condition may be carried into effect by the usual process of scutching, hackling, drawing, or any or all of the operations employed in the preparation of ramie, hemp, sisal, flax and other forms of fibre, wherein the staple or length of the fibre is greater than in some of the other natural fibres.

In carrying the invention into practical effect, it is preferable to employ fibres of long staple, but in some instances relatively short fibres may be mixed in with the long fibres.

In order that the fibres may serve efficiently to reinforce the fabric, it is desirable that they shall extend in general parallel condition and in substantially straight condition. However, the fibres have a tendency to kink or curl or otherwise depart from substantially straight condition. This fact, together with the fact that a multiplicity of the fibres are employed in sheet form for reinforcing effect, have made it difficult to so control the fibres that they will be properly distributed so as to furnish the desired reinforcement throughout the area of the fabric.

One good method of applying the unspun fibres to paper or other fabrics is characterized by supplying the fibres in the form of a series of rovings placed side by side, and feeding the rovings between fluted rolls which tends to flatten the same out into sheet form. The layer or sheet of unspun fibres may be then fed to a combing apparatus which may be operated at a speed such that the fibres are drawn out and placed

under a draft or tension such that they tend to approach substantial parallel relation. 55 Also, this combing step tends to attenuate the sheet so that the thickness of the sheet may be substantially equal to the thickness of a single fibre, and the draft or tension preferably is maintained upon the fibres 60 while they are adhesively secured to the fabric to be reenforced.

It is inevitable, however, in thus controlling the multiplicity of fibres without positive control thereover, that substantial longitudinal spaces may occur between the fibres or between groups of the fibres, and also since the fibres may be of different lengths with different draft effect thereon, the fibres may be so drawn that end to end spaces will 70 occur between some of them.

The layer or sheet of fibres thus prepared may be applied to an adhesive coating, such, for example, as black asphaltum on a single sheet of paper or fabric, and in some instances, a second sheet of paper may be superposed upon the first sheet, so that the adhesive layer and the unspun fibres therein will be covered on both sides by the paper 75 or fabric layers.

This constitutes a good efficient form of fabric for many purposes, but in some uses it is desirable that the paper or fabric shall receive reinforcement by the fibres substantially throughout the entire area thereof. 85 In other words, it is desirable that the longitudinal and end to end spaces referred to, or other spaces between the fibres shall have adequate reinforcement.

The aim and purpose of the present invention, therefore, is to provide a fabric which will employ unspun fibres as the reinforcing means therefor, and to so distribute the fibres that the liability of occurrence of the objectionable spaces referred to, will be reduced to a minimum. To accomplish this, in the present instance, a second sheet of unspun fibres such as described, is included in the composite fabric. The second sheet of unspun fibres may be desirably applied to the opposite side of one of the sheets of paper or fabric referred to, having the sheet of unspun fibres applied thereto, and the second sheet of unspun fibres may be applied to an adhesive coating or layer on such sheet of paper or fabric, and this adhesive 95 100 105

- may be black asphaltum or other appropriate adhesive. To protect and conceal the second sheet of unspun fibres, the composite paper or fabric may desirably include a 5 third sheet of paper which will be superposed on the first two sheets, and be in adhesive engagement with the adhesive layer which serves to secure the unspun fibres to the first two sheets described.
- 10 It is found in practice that where a second sheet of unspun fibres such as described is employed, that there may be longitudinal and end to end spaces therebetween, but the likelihood of registration of the spaces between the fibres of the second sheet with the 15 spaces between the fibres of the first sheet is quite remote, and as a consequence, a composite fabric provided with the two sheets of unspun fibres will substantially insure such distribution of the unspun fibres as to prevent occurrence of substantial portions of the fabric without unspun fibre reinforcement.
- 20 If a still stronger reinforcement is desired, still another sheet of unspun fibres may be employed, and if desired still another sheet of paper may be employed to conceal the unspun fibre sheet. In fact, as many more than two sheets of unspun fibres in the composite fabric may be employed as desired.
- 25 The accompanying drawing illustrates a composite sheet of fabric reenforced by unspun fibres in accordance with the present invention, and also shows several uses for which such a strip is well adapted, but it will be apparent that a fabric constructed in accordance with this invention is well adapted for various purposes other than herein shown and described.
- 30 In the drawing:
- 35 Fig. 1 is a perspective view of a strip of reenforced fabric constructed in accordance with the invention, the strips of which the same is constructed being shown rolled back at one edge;
- 40 Fig. 1<sup>a</sup> is a sectional view, on an enlarged scale, taken on the line 1<sup>a</sup>—1<sup>a</sup> of Fig. 1;
- 45 Fig. 2 is a view showing one use for which the strip of reenforced fabric is well adapted;
- 50 Fig. 3 is a view showing a somewhat different use of the same; and
- 55 Fig. 4 is a view showing still a third use for which the reenforced strip is well adapted.
- 60 Referring to the drawing and more particularly to Figs. 1 and 1<sup>a</sup>, the numeral 10 designates a strip of reenforced fabric constructed in accordance with the invention, and this reenforced strip is preferably formed of at least three separate strips of paper or other fabric designated as 11, 12 and 13. The adjacent faces of these three strips preferably have placed between the 65 same a sheet of longitudinally extending filaments of unspun fibres as designated by 14. These filaments are preferably arranged to form sheets with the individual fibres lying closely adjacent to each other in substantially parallel relation, and are secured to the adjacent faces of said strips by an adhesive, which serves also to secure the adjacent strips together, that is, the adhesive which secures the fibres upon the upper face of the strip 12 will serve also to secure the strip 11 thereto while the adhesive which secures the fibres to the lower face of the strip 12 will serve also to secure the strip 13 thereto. Any suitable adhesive may be used for this purpose, but in order that the strength of the wrapping strip 10 will not be materially affected by rain, dampness or other moisture, it is desirable that a waterproof adhesive be used, such as black asphaltum.
- 70 Various kinds of filaments of unspun fibre may be used to reinforce the strip 10, but a relatively long inexpensive filament possessing considerable strength is preferable, and since it is practically immaterial whether the fibres are coarse or not, hemp, jute, ramie, sisal, and various other well known fibres may be used as the reinforcing filament. It will also be apparent that the reinforcing filaments may be applied either to the opposite faces of the intermediate strip 12 or to the inner faces of the strips 11 and 13, and in the particular embodiment illustrated it will be noted that some fibres are shown as adhering to each of these three strips.
- 75 Since the filaments used in reinforcing the strip 10 preferably are unspun fibres, the individual fibres which are placed upon the strip to be reenforced will not in all probability be arranged uniformly upon the same, due to the tendency of the individual fibres to kink or curl, and due to the various other difficulties met with in attempting to arrange the individual fibres into a uniform sheet. As a result, small spaces or patches will probably occur upon each strip such as indicated by 14<sup>a</sup> which are not reenforced by any fibres. It is therefore very desirable to use a second strip which is similarly reenforced by a second sheet of unspun fibres, or to apply a similar reinforcing sheet of fibres to the opposite face of the strip which was previously reenforced. This is desirable because by providing two separate sheets of reinforcing filaments, as shown, it is very unlikely that these spaces or patches 14<sup>a</sup> which are not reenforced upon one sheet will fall opposite a similar patch or space upon a second sheet. It will, therefore, be seen that by providing a strip of paper of several ply having more than one sheet of reinforcing filaments, the strength of the strip which is reenforced in this manner will be practically uniform throughout.
- 80
- 85
- 90
- 95
- 100
- 105
- 110
- 115
- 120
- 125
- 130

the same, notwithstanding the fact that small spaces or gaps may occur in each sheet of filament in which the fibres are missing.

A fabric reenforced in the manner just described may be employed for many purposes. One important field of use is as a wrapper for tires, coils of wire, or an assemblage or stack of either. When a strip of fabric or paper is employed for the use just mentioned it is desirable to wrap this strip spirally about an individual tire or other ring like article, or to wrap the same spirally about the inner and outer walls of a stack of these articles to bind the same into a package.

Heretofore paper strips have been used to wrap about a single tire, or other articles which did not place a severe strain upon strip, but if the package to be wrapped was a heavy coil of wire or other heavy article, it was customary to use strips of burlap to wrap about the same, as paper heretofore used was not strong enough to withstand the severe strain and wear upon the same. While burlap usually possesses the desired strength, it is comparatively expensive and is not entirely satisfactory for other reasons.

When a strip of reenforced fabric is wound spirally about a tire, a coil of wire or other ring like article to be protected, the greatest wear upon this wrapping strip falls upon the leading or exposed longitudinally extending edge of the same, and in order to strengthen or reinforce this leading edge, a portion of the same is preferably folded under or back upon the strip, as indicated by 15 in Figs. 1 to 4 inclusive. The folding under of this edge very effectively reinforces the same, and it is found in actual use that a strip which has been reenforced by unspun fibres in the manner above pointed out and then had the leading edge of the same folded under, is strong enough to readily withstand all strains to which the same will be submitted in either winding the strip about the article to be wrapped or, later on, in transportation of the article protected by this wrapper. This is because folding the leading edge of the strip under, not only provides a smooth edge where the wear and strain is the greatest, but what is more important a very strongly reenforced edge is provided as clearly shown in Fig. 1<sup>a</sup>. In this figure it will be seen that this edge is strengthened by four sheets of unspun fibres as indicated by 14, and six sheets of paper or other fabric as indicated by 11, 12 and 13. If spaces, weak spots or areas without reinforcing fibres should occur in one of the reinforcing sheets 14 at the fold, this weak spot will invariably be reenforced by fibres at the fold in the adjacent sheet 14. Margins of different widths may be folded under as desired, but fibres will invariably fall at the folded edge.

The edge 15 of the strip 10 may be folded over in a final step in manufacturing the strip preparatory to forming this strip into a package to be sent out on the market, or, if desired, the machine used to coil this strip 70 spirally about the ring like article to be wrapped may be provided with a device for folding over this edge. The folding of the strip immediately before the same is wrapped about the article to be protected, 75 will be found desirable in most cases, because this avoids the necessity of forming a package of the strip 10 in which one edge of the same, due to the fold 15, is twice as thick as the opposite edge. Any appropriate folder of well known construction may be used to fold over this edge, either before the strip is formed into a package or while the strip is being delivered to the mechanism which winds the same about the 80 article to be wrapped.

A strip 10, when constructed in the manner above pointed out, is admirably well adapted as a wrapper to be wound spirally around one or more automobile tires, such 90 as indicated by 16 in Fig. 2, or to bind up and protect a relatively large heavy coil of wire, such as indicated by 17 in Fig. 3. These coils of wire commonly weigh over two hundred pounds and yet a wrapping 95 strip of paper when constructed in the manner above pointed out will satisfactorily withstand the strain to which it is submitted in binding up a coil of this weight. In Figs. 2 and 3 the strip 10 is shown as wound 100 spirally around more than half of the ring-like articles upon which the same is placed, and in each of these figures the leading end 18 is shown in a downwardly extending position ready to be further coiled about 105 the article which it is to cover. In each of these figures the folded over edge 15 is clearly shown in full lines upon the end portion 18 and in dotted lines where the strip 10 has been coiled.

In Fig. 4 is shown a stack of tires or other ring like articles 19 such as heretofore have been bound into a package by winding spiral strips of burlap about the same in the manner above mentioned. In the present 115 invention these articles 19 are shown as bound together by the reenforced wrapper strip 10 which is passed about the ends of the cylinder-like structure thus formed and about the inner and outer walls of the same. 120 The strip 10, when constructed as above pointed out, is sufficiently strong to secure a number of tires or other articles together in a single package, while at the same time it is much less expensive than the binding 125 strips heretofore used.

The reenforced strip 10 while shown and described as of three-ply may be reenforced with additional strips, if desired, but the particular construction shown is found to 130

be very satisfactory, due to the two separate sheets of reinforcing filaments of unspun fibres, since in this arrangement, when a space occurs upon one strip in which the reinforcing fibres are missing, the reinforcing fibres upon the other strip will, in all probability, extend over this weak spot, as it is very unlikely that two such weak spaces will fall opposite each other.

10 An important advantage in using unspun fibres to reinforce paper instead of spun fibres results from the fact that spun fibres will stretch sufficiently to permit the paper to tear before the spun fibres are broken, but 15 unspun fibres will not stretch appreciably and hence will not permit the paper to tear until the strain is great enough to break the fibres.

Claims—

20 1. As an article of manufacture, reenforced paper comprising a centre strip of paper, reinforcing layers of unspun fibres adhesively secured to the opposite faces of said centre strip with the fibres extending in substantially parallel relation, the individual fibres of each reinforcing layer being arranged closely adjacent but unsymmetrical relative to each other and the fibres in one layer serving to reinforce the spaces in 25 which fibres may be missing from the other layer, and exterior strips of paper enclosing the centre strip and the reinforcing fibres and adhesively secured thereto.

30 2. As an article of manufacture, a reenforced paper comprising a centre strip of paper, a layer of unspun fibres adhesively secured to one face of said strip and extending longitudinally of the strip, a layer of unspun fibres adhesively secured to the 35 opposite face of said strip and extending longitudinally thereof, each layer having the fibres forming the same spread approximately uniformly throughout the layer and in closely adjacent relation, and exterior 40 strips of paper enclosing the centre strip and the reinforcing unspun fibres and adhesively secured thereto.

45 3. As an article of manufacture, reenforced paper comprising a centre strip of paper, reinforcing layers of filaments adhesively secured to the opposite faces of said centre strip with the filaments extending in substantially parallel relation, the individual filaments of each reinforcing layer 50 being arranged closely adjacent but unsymmetrical relative to each other and the filaments in one layer serving to reinforce the spaces in which filaments may be missing from the other layer, and exterior strips 55 of paper enclosing the centre strip and the reinforcing filaments secured to the centre strip.

60 4. As an article of manufacture, a wrapper strip of reenforced paper comprising a centre strip of paper, longitudinally ex-

tending unspun fibres adhesively secured to each surface of the centre strip of paper in the form of a thin sheet or layer, exterior strips of paper enclosing the central strip and the reinforcing unspun fibres and adhesively secured thereto, and the reenforced paper having a longitudinally extending edge thereof folded under to further strengthen the same.

5. A wrapper strip of reenforced paper to be wound spirally about ring like articles of manufacture, comprising a three-ply strip of paper having the adjacent faces of the individual strips reenforced by longitudinally extending filaments of relatively long, strong, unspun fibres secured to said faces by a waterproof adhesive of black asphaltum, said wrapper strip having the leading longitudinally extending edge thereof further strengthened by folding a portion of the same under.

6. A wrapper strip of reenforced paper to be wound spirally about ring like articles of manufacture, comprising a three-ply strip of paper reenforced by longitudinally extending filaments of unspun fibres adhesively secured to the opposite faces of the intermediate strip, said three-ply strip having the longitudinally extending edge thereof of which is exposed when wound spirally about a ring like article further reenforced by folding a portion of the same under.

7. A wrapper strip of reenforced paper, comprising a strip of paper having a layer of unspun fibres adhesively secured to each of its faces, each layer of unspun fibres having a strip of paper adhesively secured to the outer face thereof, said reenforced paper having a longitudinally extending edge thereof folded under to further strengthen the same.

8. As an article of manufacture, a reenforced paper wrapper comprising a centre strip of paper, longitudinally extending unspun fibres adhesively secured to each surface of the centre strip of paper in the form of a thin layer, and exterior strips of paper inclosing the central strip and the reinforcing unspun fibres and adhesively secured thereto.

9. As an article of manufacture, reenforced paper comprising a centre strip of paper, a series of unspun fibres adhesively secured to each face of said strip in substantially parallel relation and under lengthwise tension, and exterior strips of paper enclosing the centre strip and the reinforcing fibres adhesively secured to the centre strip.

10. As an article of manufacture, reenforced paper comprising a centre strip of paper, reinforcing layers of unspun fibres adhesively secured to the opposite faces of said centre strip with the fibres extending in substantially parallel relation and each

layer having a thickness substantially equal to the thickness of one of the fibres, and exterior strips of paper enclosing the centre strip and the reinforcing fibres secured to the centre strip.

11. A wrapper strip of reenforced paper to be wound spirally about articles of manufacture, comprising a three-ply strip of paper having the adjacent faces of the in-

dividual strips reenforced by longitudinally extending filaments secured to said faces by a waterproof adhesive, and the wrapper strip having one of its longitudinal edges further strengthened by folding a portion of the same under.

In testimony whereof, I have signed my name to this specification.

CHARLES H. HOWARD.